

S. E. FINLEY,  
METHOD OF TREATING ROADWAYS,  
APPLICATION FILED FEB. 15, 1915.

1,192,178.

Patented July 25, 1916.

1. A priming coat containing volatile matter of slow diffusion.  
2. A confining coat therefor.



Inventor:  
Sam C. Finley  
by Paul Goldsmith Atty

# UNITED STATES PATENT OFFICE.

SAM EVERETT FINLEY, OF ATLANTA, GEORGIA.

## METHOD OF TREATING ROADWAYS.

1,192,178.

Specification of Letters Patent. Patented July 25, 1916.

Application filed February 15, 1915. Serial No. 8,370.

To all whom it may concern:

Be it known that I, SAM E. FINLEY, a citizen of the United States, residing at Atlanta, county of Fulton, and State of Georgia, have 5 invented certain new and useful Improvements in Methods of Treating Roadways; and I do hereby declare the following to be a full, clear, and exact description of the invention, such as will enable others skilled in 10 the art to which it appertains to make and use the same.

This invention relates to the surface treatment of roadways, and has for its object to provide the novel method of treating road- 15 ways, hereinafter described.

It has been found in practice that when a roadway is treated with heavy bituminous products, for the purpose of preserving the road surface and rendering the same wear- 20 resisting, the bituminous products cannot be made to bond or unite with the particles of the roadway, as there is always a sufficient amount of dust and loose particles adhering to the stone to act as a separator between the 25 stone proper and the heavy bitumen. This is true, regardless of how carefully the stone may be crushed or graded. This condition not only exists in "penetration macadam" roadways, but also exists in concrete roads 30 or streets constructed either by tamping or floating with a trowel. When concrete roads are so constructed, there will come to the surface a portion of sand and cement which will probably have sufficient cementing 35 values to hold them together, but this portion of the sand so brought to the surface is not as rich with cement as the lower portion of the roadway, so that a thin sheet or scale at the road surface results, which is suscep- 40 tible to cracking or separating from the harder and more firmly united base portion. No matter how carefully this surface may be swept or cleaned prior to the application of a heavy bitumen, it has been found that a 45 good union cannot be obtained, as a thin film of dust or foreign matter will always remain to act as a separator between the heavy liquid bitumen and the road surface. This is also true of practically all types of road- 50 ways or street surfaces, including roads constructed of gravel, water-bound macadam and the like. A lighter bitumen, however, will penetrate the above-mentioned film of dust, but a light bitumen does not possess the 55 necessary preserving and cementing values, as it contains a high percentage of volatile

matter and only a low percentage of cementing value. This light bitumen has as its greatest asset, the ability to suppress dust, but is of little value in preserving the roadway and rendering the same wear-resisting. In fact, it has been found that it often happens that considerable disintegration takes place in the portion of the roadway treated with light bituminous products, for the reason that the light oils volatilize and leave the treated portion of the roadway in the form of a coating in which the natural bonding or cementing values of the material are destroyed.

The present invention contemplates the use of both the heavy and light bituminous products in such a way as to combine their advantageous qualities, and to dispense with the above-named objectionable effects involved in the individual use of each. After a great deal of experimenting, it has been found that the lighter materials may be utilized to great advantage when correctly used in combination with the heavier materials, and a much better road surface produced than can be obtained by the individual use of either of the products. The present invention, therefore, contemplates the treatment of the roadway whether the same be of 85 concrete, bituminous macadam, sheet asphalt, stone, gravel, or other construction, with a lighter grade of bitumen which penetrates the roadway and is not prevented from doing so by the existence of dust or 90 foreign matter. At a suitable time after the treatment of the roadway with the lighter bitumen, a heavy bitumen is applied, which firmly unites with the lighter bitumen, and is in this way bonded or cemented with the 95 particles of the roadway. The lighter bitumen, therefore, serves as a priming coat which permits the use of the heavier bituminous products having wear-resisting and other properties not possessed by the lighter 100 bituminous products. This priming coat of lighter bituminous products, therefore, serves the same purpose as the priming coat in painting wood or the like, where it is necessary to apply a priming coat of thin paint before 105 the wood or other surface treated will receive the heavier final coat of paint. The priming coat possesses penetrating qualities which the heavier coat does not possess.

In addition to the above results produced 110 by the use of the so-called priming coat of bitumen, the lighter bitumen penetrates

deep into the roadway, and it is retained there by the heavier surface bitumen, which has the following beneficial action upon the roadway. The lighter bitumen contains a great deal of volatile matter, but the heavier bituminous coating which has a low percentage of volatile matter serves as a seal, and prevents the escape of the volatile matters of the underlying coating of light bituminous matter. As the volatile matters in the lighter bitumen cannot escape, the tendency is for them to penetrate farther and farther into the roadway, and in so doing, a chemical action results imparting a new life to the roadway, and a higher cementing value to the priming coat than it originally possessed. The disintegrating action caused by the volatilization of the lighter bitumen is, therefore, prevented, as the heavier coating prevents escape of the volatile matter. The result is that a hard and elastic road surface is produced which has been found in practice to be superior to all types of roadways treated by similar methods. If a portion of the volatile matter so confined beneath the heavy bituminous coating works upward instead of downward into the roadway, it will be absorbed by the finishing coat of heavy bitumen and act thereupon in a manner similar to what is commonly termed a "cut-back", that is to say, it will make the heavy bitumen more of a liquid, and this chemical action will result in carrying the heavier or finishing coat farther into the road surface, so that its cementive value may be utilized below the original road surface. This action takes place so slowly that practically none of the volatile oils of the priming coat are lost, whereas, if the lighter bitumen is used by itself without the heavier finishing coat, it loses over half of its lighter constituents by volatilization within sixty to ninety days.

In carrying out the method, it has been found desirable for the best results to first sweep the road surface as free as possible from all loose material, and then apply the lighter bitumen by any suitable means, the quantity applied depending upon the absorption qualities of the roadway. The quantity applied should be limited to the amount that the road surface is capable of absorbing. In some instances, it may be desirable to then apply a thin layer of sand, stone screenings, or sweepings from the road or street surface, and open the roadway to traffic and exposure to the elements. The heavier coating of bituminous material may then be applied to the road surface, but preferably the application of the heavier bitumen is made just after the application of the priming coat of lighter bitumen. The second coat of heavier bituminous material may, if desired, be covered with a layer of either sand, fine gravel, or crushed stone.

The lighter bitumen not only serves to penetrate into the body of the roadway, and thereby act as a priming coat for the heavier bitumen, but also produces other beneficial results, due to the fact that its volatile matters are confined within the roadway by the heavier bituminous finishing coat. The heavier bituminous coating which would not be bonded and firmly united with the roadway, if it were not for the relatively light priming coat, produces the elastic wear-resisting surface, as the heavier bituminous products possess the cementing and wear-resisting qualities which the lighter products do not possess, and which it is essential that the top dressing should possess. There is, therefore, an intimate co-operation between the two layers of bituminous material, as each serves to permit the use of the other, and when used in combination, their beneficial characteristics are retained, whereas the disadvantages accompanying the individual use of either of the materials independent of the other are overcome.

In the construction of "penetration macadam" roadways, after a layer of coarse stone has been applied and rolled, and then a wearing surface of stone applied to the first layer and rolled, it has been the custom to apply a very heavy binder which required heating to a temperature of from 300° to 400° F. Obviously, a binder requiring such a high heating soon thickens and the thin film of dirt which necessarily remains on the surface of the broken stone will act as a separator to prevent a union between the heavy binder and the stone. This objection is overcome by the present method, as the broken stone may first be treated with the penetrating and priming coat of light and unheated bitumen which unites with the stone and prepares the same for receiving the heavy heated bitumen, which latter will then firmly unite with the priming bitumen, and hence the broken stone.

The accompanying drawing illustrates in transverse vertical section, a portion of a water-bound macadam roadway constructed in accordance with my improved method. This type of roadway is illustrated merely for exemplary purposes, it being understood that the method is applicable to many other types.

The portion of the road-bed indicated at A shows the condition of the same before treatment. That portion indicated at B has had the above described priming coat applied thereto, the material of the priming coat being represented at 1. Due to the high penetrating value of the material of the priming coat, it is readily absorbed by the surface of the roadway, as above stated. That portion of the road-bed indicated at

C shows the condition of the same after the application of the heavier bituminous coating 2 which, as indicated in the drawing, firmly adheres to the road-bed on account of 5 the provision of the priming coat.

The hereinbefore described "cutting-back" action of the priming coat 1 on the heavier bituminous coating 2 and the consequent carrying of a portion of the heavier coating 10 down into the heart of the road-bed is represented in the drawing, in section C. In this part of the drawing, it will be noted that the portion of the top coating cut back by the priming coat is carried by the priming coat deep into the heart of the road-bed, where its cementive value may be utilized. This is a result of the retention of the gases or volatile matter in the road-bed by the 15 heavier coating and the consequent cutting-back action which increases the penetrating value of a portion of the heavier coating, and, therefore, the priming coat and the cutting-back portion of the heavier coat penetrate deep into the roadway, as illustrated 20 in the drawing and as hereinbefore described.

What I claim is:—

1. The method of treating road-beds which consists in applying to the road surface a penetrating and priming coat of light 25 bituminous substance containing a large percentage of volatile matters capable of slow

diffusion, and then before the volatile matters escape, applying a coat of heavier bituminous substance capable of confining and retaining the volatile matters in the road bed, the priming coat being capable of binding the top coat to the road surface and of gradually cutting back the same to utilize its cementive value below the original road surface. 35

2. The method of treating road-beds which consists in first removing the loose dust from the road surface, applying to the cleaned road surface a penetrating and priming coat of light bituminous substance 40 containing a large percentage of volatile matters capable of slow diffusion, and then before the volatile matters escape, applying a coat of heavier bituminous substance capable of confining and retaining the volatile matters in the road bed, the priming coat being capable of binding the top coat to the road surface and of gradually cutting back the same to utilize its cementive value below the original road surface. 45

In testimony whereof I affix my signature, in presence of two witnesses.

SAM EVERETT FINLEY.

Witnesses:

H. F. SMITH,  
HUGH CRISWELL.